

R. J. PIERSOL,  
PROCESS AND APPARATUS FOR METAL PLATING,  
APPLICATION FILED JAN. 3, 1920.

1,343,842.

Patented June 15, 1920.

Fig. 1,



Fig. 2.



WITNESSES

Edw. Thorpe  
L.A. Paley

INVENTOR

ROBERT J. PIERSOL.  
BY *Munro Co.*  
ATTORNEYS

# UNITED STATES PATENT OFFICE.

ROBERT J. PIERSOL, OF BENTLEYVILLE, PENNSYLVANIA.

## PROCESS AND APPARATUS FOR METAL-PLATING.

1,343,842.

Specification of Letters Patent. Patented June 15, 1920.

Application filed January 3, 1920. Serial No. 349,172.

To all whom it may concern:

Be it known that I, ROBERT J. PIERSOL, a citizen of the United States, and a resident of Bentleyville, county of Washington, and State of Pennsylvania, have invented a new and Improved Process and Apparatus for Metal-Plating, of which the following is a full, clear, and exact description.

This invention relates to means for plating one material with another and has reference more particularly to a means for plating *in vacuo* at a temperature between the melting point of the two materials, the material of the higher melting point with the material of the lower melting point.

The object of this invention is to provide a means for plating one metal with another metal which will be inexpensive and easy to apply.

Many materials, such as iron and copper, cannot be plated successfully the one with the other, by ordinary means, because an inhibitory gaseous film between the two metals interferes with adhesion. Experiment has shown that when plating takes place in a vacuum, the higher temperature breaks down the gaseous film which is removed by the vacuum. For instance, iron can be plated successfully with melted copper *in vacuo*. But unless the gaseous film had been removed by the vacuum the adhesion would have been imperfect. This is probably due to the fact that the metal has greater adhesion for the gaseous film than it does for the other metal. Since this is true, necessarily the film must be removed before the influence of the adhesive attraction of the two metals can come into play. Experiment has shown that when the gaseous films are removed, two different materials, other than iron and copper, may be plated with each other in the same way. Therefore this process covers any two materials for which adhesion is desired.

I have knowledge that processes have been used in which a solid material is covered by a material which has been volatilized *in vacuo*. But a volatilized material is in a gaseous state instead of a liquid state. Therefore there is no relation between the two processes. The previous processes have had to do with coating a material in a solid state by a material in a gaseous state. While my process has to do with coating a material

in a solid state by a material in a liquid state.

Such a process is of commercial importance. For instance a piece of statuary of an inexpensive base, either metal or non-metal, could be coated with copper with a slight expense. But the copper plated statue would have all the durability and beauty of a solid copper statue. Also metals, such as steel, which may be corroded by weathering, could be copper plated, thereby increasing their life many fold.

Reference is to be had to the accompanying drawing forming a part of this specification in which it is understood that the drawing illustrates only one form of apparatus which could be used in carrying out my process, and in which

Figure 1 is a central sectional view through the apparatus.

Fig. 2 is a sectional view on the line 2—2 of Fig. 1.

Referring to the accompanying drawing by numerals, 10 indicates a vacuum jar which may be placed in an oven at a temperature between the melting points of iron and copper. 11 is an exhaust pipe which is attached to any suitable vacuum pump not shown. A crucible 12 is placed in said vacuum jar and contains melted copper 13. A block of iron 14 is suspended on a wire 15 above said crucible, said wire being wound around and secured to a pulley 16 fixed to a shaft 17. The shaft 17 is rotatably supported by bearings 18 and 19 constructed in any suitable manner in the walls of the vacuum jar 10. A chamber 20 preferably cylindrical in shape is interposed between the bearing 18 and the vacuum jar 10, and a soft iron core 21 is fixed to the shaft 17 and positioned in said chamber 20. The iron core 21 has a plurality of radiating arms each of which is attracted magnetically by an electro-magnet 22, said electro-magnets being arranged in series in a circuit 23 which includes a battery 24. These electro-magnets may be rotated about the chamber 20 so that the arms of the iron core 21 will follow their movement and thus the vertical position of the block of iron 14 may be changed. A door 23 is fixed to the vacuum jar 10 by means of bolts 24, and is adapted to cover an opening 25 in said vacuum jar. This door 23 may be easily removed and a new

object to be plated can be attached to the wire 15.

I would state in conclusion that the invention has to do primarily with a process and the drawing shows only one of numerous ways by which the mechanical part of the process may be carried on, so that the field covering the process should not be limited by any one type of apparatus. Also the process should cover any two different metals whatsoever and should not be limited to the two already mentioned in illustration.

Having thus described my invention, I claim as new and desire to secure by Letters

15 Patent:

1. A process for the plating of one metal by another metal which consists in treating one of said metals with the other of said metals *in vacuo* at a temperature between 20 the melting points of the two metals.

2. A process for the plating of one metal with another metal which consists in enveloping the metal with the higher melting point by the fused bath of the metal with 25 the lower melting point, said metals being heated *in vacuo* to a temperature between their melting points.

3. An apparatus for the plating of one material with another material which consists in a vacuum jar, a container placed in

said jar adapted to contain a fused material, and means for lowering a second material into the first mentioned fused material.

4. An apparatus for the plating of one material with another material which consists in a vacuum jar, a container placed in 35 said jar adapted to contain a fused material, a solid material, a shaft rotatably mounted inside said vacuum jar, a flexible means connecting said solid material and said shaft 40 adapted to wind upon said shaft as said shaft is rotated, and means for rotating said shaft.

5. An apparatus for the plating of one material with another material which consists in a vacuum jar, a container placed in 45 said jar adapted to contain a fused material, a solid material, a shaft rotatably mounted inside said vacuum jar, a flexible means connecting said solid material and said shaft 50 adapted to wind upon said shaft as said shaft is rotated, a plurality of radiating soft iron arms fixed to said shaft, a plurality of electromagnets rotatably mounted outside said vacuum jar adapted to magnetically engage the soft iron arms inside said vacuum jar and rotate said arms and said shaft when said electro magnet is rotated, and means for electrically exciting said electromagnets.

ROBERT J. PIERSÖL.